# EUROPEAN PATENT SPECIFICATION

(11) **EP 2 117 280 B1**
(45) Date of publication and mention of the grant of the patent: **11.04.2018**
(21) Application number: 08711793.3
(22) Date of filing: 22.02.2008
(51) Int. Cl.: H05B 3/18, F23Q 7/00, H05B 3/10, H05B 3/48

(54) **CERAMIC HEATER, GLOW PLUG USING THE CERAMIC HEATER, AND CERAMIC HEATER MANUFACTURING METHOD**
KERAMISCHES HEIZELEMENT, DAS KERAMISCHE HEIZELEMENT VERWENDENDE GLÜHKERZE UND VERFAHREN ZUR HERSTELLUNG EINES KERAMISCHEN HEIZELEMENTS
DISPOSITIF DE CHAUFFAGE EN CERAMIQUE, BOUGIE DE PRECHAUFFAGE UTILISANT LE DISPOSITIF DE CHAUFFAGE EN CERAMIQUE, ET PROCEDE DE FABRICATION DU DISPOSITIF DE CHAUFFAGE EN CERAMIQUE

(30) Priority: 22.02.2007 JP 2007041681
(43) Date of publication of application: 11.11.2009
(73) Proprietor: Kyocera Corporation, Kyoto-shi Kyoto 612-8501 (JP)
(72) Inventor: HIURA, Norimitsu, Kirishima-shi Kagoshima 899-4396 (JP)
(74) Representative: Viering, Jentschura & Partner mbB Patent- und Rechtsanwälte
(86) International application number: PCT/JP2008/053019
(87) International publication number: WO 2008/105327

(56) References cited:
- EP-A2- 1 248 045
- JP-A- 03 149 791
- JP-A- 07 239 126
- JP-U- H0 543 495
- JP-U- 05 043 495

## Description

### Technical Field

The present invention relates to ceramic heaters used as, for example, ignition heaters, flame detection heaters, sensor heaters, and heating heaters. The ignition heaters and the flame detection heaters are used in the form of, for example, combustion devices such as combustion-type car heaters and kerosene fan heaters. The sensor heaters are used in, for example, automotive glow plugs and various sensors such as oxygen sensors. The heating heaters are used in, for example, measuring instruments.

### Background Art

A ceramic heater usually has a structure in which a heat-generating resistor and leads for feeding are arranged in a ceramic body. The ceramic heater is manufactured in such a manner that the heat-generating resistor and the leads are separately formed, arranged to partly overlap with each other, and then fired together with the ceramic body.

EP 1 248 045 A2 discloses a ceramic heater provided with an insulating ceramic substrate, a resistance heating element buried in the insulating ceramic substrate, and an ion current detecting electrode portion formed integrally with the resistance heating element in the insulating ceramic substrate and having its own surface portion exposed as an ion current detecting face to the surface of the insulating ceramic substrate.

JP H05 43495 U discloses a ceramic heater comprising a heat-generating resistor, a lead configured for supplying power to the heat-generating resistor, and a ceramic body containing the heat-generating resistor and the lead therein. The heat-generating resistor comprises a connecting portion being connected to the lead and having a width less than the width of the lead, and a main heat-generating portion other than the connecting portion.

### Disclosure of Invention

### Problems to be Solved by the Invention

In the manufacture of a ceramic heater, a heat-generating resistor 3 is significantly misaligned with leads 5 or the stress applied thereto causes bumps 3c on the heat-generating resistor 3 as shown in Figs. 11A and 11B. When the bumps 3c have a sharp wedge shape, the bumps possibly causes cracks and/or the like in the heat-generating resistor and the leads.

The present invention has been made to solve the above problem. It is an object of the present invention to provide a ceramic heater in which the formation of such bumps are reduced and therefore cracks are reduced from being formed in a heat-generating resistor, leads, or a ceramic body.

### Means for Solving the Problems

A ceramic heater according to the present invention comprising a heat-generating resistor, configured for supplying power to the heat-generating resistor, a ceramic body containing the heat-generating resistor and the lead therein. The heat-generating resistor comprises a connecting portion being connected to the lead and having a width less than the width of the lead, and a main heat-generating portion other than the connecting portion. The lead comprises a recessed portion being located at end portion of the lead, being connected to the connecting portion, and being open at an only one side of the longitudinal direction of the lead and an only one side of the thickness direction of the lead. At least a part of the connecting portion is located inside the recessed portion. Advantages

In a ceramic heater according to the present invention, at least a part of connecting portion is located inside the recessed portion; hence, protrusion of the connecting portion is controlled. This is effective in that concentration of thermal stress on a single site is controlled during rapid heating or cooling or during firing or usage. A possibility of the formation of a crack is reduced in the heat-generating resistor, the lead, or a ceramic body near junctions between a heat-generating resistor and the lead. Therefore, the ceramic heater can be provided so as to be excellent in durability and reliability.

### Best Modes for Carrying Out the Invention

Ceramic heaters according to embodiments of the present invention will now be described with reference to the accompanying drawings.

As shown in Figs. 1 to 3, a ceramic heater 1 (hereinafter also referred to as the heater 1) according to a first embodiment of the present invention comprises a heat-generating resistor 3, lead 5 configured for supplying power to the heat-generating resistor 3, and a ceramic body 7 containing the heat-generating resistor 3 and the lead 5 therein. The heat-generating resistor 3 comprises connecting portion 3a being connected to the lead 5 and having a width less than the width of the lead 5, and a main heat-generating portion 3b other than the connecting portion 3a. The lead 5 comprises a recessed portion 9 being located at end portion of the lead 5, being connected to the connecting portion 3a, and being open at an only one side of the longitudinal direction of the lead 5 and an only one side of thickness direction of the lead 5. At least a part of the connecting portion 3a is located inside the recessed portion 9.

In this embodiment, a longitudinal direction, a thickness direction, and a width direction are defined as described below. The longitudinal direction is defined as a direction that connects one end of lead, which extends substantially linearly, and the other end and that is parallel to the lead as shown in Fig. 1. The width direction is defined as a direction that connects the centers of the leads 5, which are adjacent to each other, in cross section that is perpendicular to the longitudinal direction and includes junctions between the connecting portion 3a and the lead 5 as shown in Fig. 2A. The thickness direction is defined as a direction that is perpendicular to the width direction and the longitudinal direction.

In this embodiment, a thickness and a width mean a length in the thickness direction and a length in the width direction, respectively. The depth D of each recessed portion 9 is defined as the maximum length, in the thickness direction, between a surface portion of the recessed portion 9 and a line connecting two peaks X sandwiching the recessed portion 9 as shown in Fig. 2B, the two peaks X being portions of a corresponding one of the lead 5.

In the heater 1 of this embodiment, the lead 5 comprises a recessed portion 9 being open at an only one side of the longitudinal direction of the lead 5 and an only one side of the thickness direction of the lead 5. And at least a part of the connecting portion 3a is located in the recessed portion 9. This results in that a formation of bump on portion of the heat generating resister 3, which is connected to the leads 5 is controlled. Therefore, occurrence a crack as described above is controlled because it is controlled that thermal stresses concentrated on junction between the heat-generating resistor 3 and the lead 5 when the heat-generating resistor 3 and the lead 5 are rapidly heated or cooled during firing or usage.

The heat-generating resistor 3 is electrically connected to an anode-side electrode 13 and a cathode-side electrode 11 through the leads 5 and is further electrically connected to an external power supply (not shown) through the anode-side electrode 13 and the cathode-side electrode 11. Heat can be generated from the heat-generating resistor 3 in such a manner that a voltage is applied to the heat-generating resistor 3 from the external power supply.

As shown in Fig. 1, the connecting portion 3a preferably has a width less than that of the main heat-generating portion 3b. This is because the possibility of the formation of a crack in the ceramic body 7 can be reduced. In particular, this is because the main heat-generating portion 3b can be designed to have a small thickness if the main heat-generating portion 3b is designed to have a uniform cross-sectional area and a large width such that a desired amount of heat is achieved.

The ceramic heater is generally manufactured in such a manner that a paste for forming the heat-generating resistor 3 and a paste for forming the lead 5 are sandwiched between a plurality of ceramic sheets for forming the ceramic body 7. In this embodiment, the adhesion between the ceramic sheets can be enhanced because the thickness of the main heat-generating portion 3b can be set to be small. Therefore, the possibility of the formation of a crack in the ceramic body 7 can be reduced.

In particular, the connecting portion 3a preferably has a width equal to 30% to 80% of that of the main heat-generating portion 3b. When the connecting portion 3a has a width equal to 30% or more of that of the main heat-generating portion 3b, the strength of junction between the main heat-generating portion 3b and the connecting portion 3a can be enhanced. When the connecting portion 3a has a width equal to 80% or less of that of the main heat-generating portion 3b, the adhesion between the ceramic sheets can be enhanced.

On the other hand, when the connecting portion 3a has a width equal to that of the main heat-generating portion 3b, printing yield can be increased. This is because the heat-generating resistor 3 can be formed so as to have a constant width. Since the heat-generating resistor 3 has a simple shape when having such a constant width, the whole of the heat-generating resistor 3 can be readily formed by printing. This is effective in increasing printing yield.

As shown in Fig. 3, it is effective that the connecting portion 3a has a thickness less than that of the main heat-generating portion 3b. This is because the difference between the thickness of the main heat-generating portion 3b and the thickness of the lead 5 can be reduced. Therefore, the adhesion between the main heat-generating portion 3b, the lead 5, and the ceramic body 7 can be enhanced. This results in that a separation of the main heat-generating portion 3b, the lead 5, and the ceramic body 7 can be controlled from each other.

In particular, the connecting portion 3a preferably has a thickness L2 equal to 40% to 95% of the thickness L1 of the main heat-generating portion 3b. When the connecting portion 3a has a thickness L2 equal to 40% or more of the thickness L1 of the main heat-generating portion 3b, the bonding strength between the lead 5 and the connecting portion 3a can be enhanced. When the connecting portion 3a has a thickness L2 equal to 95% or less of the thickness L1 of the main heat-generating portion 3b, the connecting portion 3a can be readily placed in the recessed portion 9. This allows the adhesion between the connecting portion 3a and lead 5 to be enhanced.

On the other hand, when the connecting portion 3a has a thickness L2 equal to the thickness L1 of the main heat-generating portion 3b, printing yield can be increased. This is because the heat-generating resistor 3 can be formed so as to have a constant thickness. Since the heat-generating resistor 3 has a simple shape when having such a constant thickness, the whole of the heat-generating resistor 3 can be readily formed by printing. This is effective in increasing printing yield.

As shown in Fig. 4, it is effective that the main heat-generating portion 3b has a thickness L1 substantially equal to the thickness L3 of the leads 5. The smaller the difference in thickness between the main heat-generating portion 3b and the lead 5, the smaller the difference in level between the main heat-generating portion 3b and the lead 5. Since there is substantially no difference in level between the main heat-generating portion 3b and the lead 5 when the main heat-generating portion 3b has a thickness L1 substantially equal to the thickness L3 of the lead 5, the main heat-generating portion 3b and the lead 5 can be readily provided in the ceramic body 7. This results in that a misalignment between the heat-generating resistor 3 and the lead 5 can be controlled. The fact that the main heat-generating portion 3b and the lead 5 have substantially the same thickness means that the difference in thickness between the main heat-generating portion 3b and the lead 5 is less than the thickness variation of the main heat-generating portion 3b and the thickness variation of the lead 5.

The connecting portion 3a preferably has a thickness less than that of the lead 5. This allows the heat-generating resistor 3 to have high resistance. The increase of the resistance of the heat-generating resistor 3 allows the main heat-generating portion 3b to efficiently generate heat and suppresses a increase the temperature of the lead 5 effectively.; hence, the durability of the ceramic heater 1 can be enhanced.

In particular, the connecting portion 3a preferably has a thickness L2 equal to 5% to 50% of the thickness L3 of the lead 5 as shown in Figs. 3 and 4. When the connecting portion 3a has a thickness L2 equal to 5% or more of the thickness L3 of the lead 5, the bonding strength between the lead 5 and the connecting portion 3a can be enhanced. When the connecting portion 3a has a thickness L2 equal to 50% or less of the thickness L3 of the lead 5, the connecting portion 3a can be stably placed in the recessed portion 9. This results in that a protrusion of the connecting portion 3a from the recessed portion 9 is controlled effectively; hence, the formation of bump on the connecting portion 3a is controlled.

The connecting portion 3a is preferably substantially quadrilateral in cross section perpendicular to the longitudinal direction as shown in Fig. 2B. When the connecting portion 3a is substantially quadrilateral in cross section, the recessed portion 9 are allowed to be large. Therefore, this result in that a protrusion of the connecting portion 3a from the recessed portion 9 is controlled; hence, the possibility of the formation of bump on the connecting portion 3a is low. This results in that the formation of a crack near the connecting portion 3a can be controlled.

The heat-generating resistor 3 may be made of a carbide, nitride, or silicide of W, Mo, or Ti as a main component. In particular, the heat-generating resistor 3 is preferably made of WC in view of the thermal expansion coefficient, heat resistance, and resistivity thereof.

The heat-generating resistor 3 preferably contains boron nitride. A conductive component contained in the heat-generating resistor 3 usually has a thermal expansion coefficient greater than that of a ceramic component, such as silicon nitride, contained in the ceramic body 7. This causes stress between the heat-generating resistor 3 and the ceramic body 7. On the other hand, boron nitride has a thermal expansion coefficient less than that of a ceramic component such as silicon nitride and hardly reacts with the conductive component in the heat-generating resistor 3. This allows the heat-generating resistor 3 to have a small thermal expansion coefficient without significantly varying heat-generating properties of the heat-generating resistor 3.

In particular, the content of boron nitride is preferably 4% to 20% by weight. When the boron nitride content is 4% by weight or more, the thermal stress generated between the heat-generating resistor 3 and the ceramic body 7 can be reduced because the heat-generating resistor 3 has a small thermal expansion coefficient.

When the boron nitride content is 20% by weight or less, varying the resistance of the heat-generating resistor 3 can be reduced. This allows the resistance of the heat-generating resistor 3 to be stable without significantly varying heat-generating properties of the heat-generating resistor 3. The boron nitride content is more preferably 12% by weight or less.

It is effective that the heat-generating resistor 3 contains the ceramic component, such as silicon nitride, contained in the ceramic body 7. When the heat-generating resistor 3 contains the ceramic component, the difference between the thermal expansion coefficient of the heat-generating resistor 3 and that of the ceramic body can be reduced. When the ceramic component is silicon nitride, the heat-generating resistor 3 preferably contains 10% to 40% by weight silicon nitride.

The leads 5 may be made of a carbide, nitride, or silicide of W, Mo, or Ti. In particular, the leads 5 are preferably made of WC in view of the thermal expansion coefficient, heat resistance, and resistivity thereof.

It is more preferred that the lead 5 be made of WC and contains 15% to 40% by weight silicon nitride. When the lead 5 contains 15% by weight or more silicon nitride, the difference between the thermal expansion coefficient of the lead 5 and the thermal expansion coefficient of the ceramic body can be reduced and therefore the formation of a crack between the lead 5 and the ceramic body can be controlled. When the lead 5 contains 40% by weight or less silicon nitride, increasing the resistance of the lead 5 can be reduced. The content of silicon nitride therein is further more preferably 20% to 35% by weight.

The lead 5 and the heat-generating resistor 3 preferably contain the same main component. This allows the adhesion between the heat-generating resistor 3 and the lead 5 to be enhanced; hence, the possibility of the formation of a crack in junction between the heat-generating resistor 3 and the lead 5 can be reduced.

The ceramic body 7 may be made of, for example, an insulating ceramic material such as an oxide ceramic material, a nitride ceramic material, or a carbide ceramic material. In particular, a ceramic material made of silicon nitride is preferably used. This is because the use of the ceramic material made of silicon nitride is effective in enhancing strength, toughness, electric insulation, and heat resistance.

Such a ceramic material can be obtained as described below. Silicon nitride, which is a main component, is mixed with 3% to 12% by weight of a rare-earth element oxide, such as Y₂O₃, Yb₂O₃, and Er₂O₃, serving as a sintering aid; 0.5% to 3% by weight Al₂O₃; and 1.5% to 5% by weight SiO₂. The mixture is formed into a predetermined shape and then fired at 1650°C to 1780°C by hot pressing.

When the ceramic body 7 contains silicon nitride, MoSiO₂ or WSi₂ is preferably dispersed therein. This allows the ceramic body 7 to have an increased thermal expansion coefficient; hence, the difference in thermal expansion coefficient between the ceramic body 7 and the heat-generating resistor 3 can be reduced. This results in that the durability of the ceramic heater 1 can be enhanced.

A second embodiment of the present invention will now be described.

In this embodiment, connecting portion 3a is trapezoidal in cross section perpendicular to the longitudinal direction as shown in Fig. 5. Since the connecting portion 3a is trapezoidal in cross section, the possibility of the formation of crack in the heat-generating resistor 3 or lead 5 can be more reduced than that described in the first embodiment. The reason for this is as described below.

The thermal expansion of a heat-generating resistor 3 causes thermal stress between the heat-generating resistor 3 and recessed portion 9 present in the lead 5. In the embodiment shown in Fig. 2A, the recessed portion 9 connected to the connecting portion 3a has side surfaces parallel to each other and therefore the directions of the thermal stresses applied to the parallel side surfaces of the recessed portion 9 are opposite to each other; hence, it is difficult to disperse the thermal stresses applied thereto. However, in this embodiment, the connecting portion 3a is trapezoidal and therefore such thermal stresses can be dispersed in the thickness direction (the vertical direction in Fig. 5). Since thermal stresses can be dispersed, the possibility of the formation of a crack in the heat generating resistor 3 and the leads 5 can be reduced.

A third embodiment of the present invention will now be described.

In this embodiment, recessed portion 9 is curved in cross section perpendicular to the width direction as shown in Fig. 6. In other words, surface of connecting portion 3a that is connected to the recessed portion 9 is curved. This prevents thermal stresses from being locally concentrated on the connecting portion 3a as compared to the first embodiment; hence, the possibility of the formation of a crack in the connecting portion 3a and the recessed portion 9 can be reduced.

In particular, the recessed portion 9 is preferably substantially arced in cross section perpendicular to the longitudinal direction shown in Figs. 7A and 7B. This allows thermal stress to be substantially uniformly dispersed; hence, thermal stresses are prevented from being locally concentrated on the connecting portion 3a. This results in that the possibility of the formation of a crack in the connecting portions 3a and the recessed portion 9 can be reduced.

A fourth embodiment of the present invention will now be described.

In the fourth embodiment, lead 5 has recessed portion 9 which are located at ends connected to two heat-generating resistors 3 and which are located at positions opposed to each other and the heat-generating resistors 3 each have connecting portions 3a partly located in the recessed portions 9 as shown in Fig. 8. Therefore, the symmetry in temperature distribution between a portion and another portion of each heat-generating resistors 3 that are spaced from each other in the thickness direction is good; hence, the temperature variation of a heater 1 in the thickness direction during usage can be reduced. This results in that a formation of a crack in the heat-generating resistor 3 is controlled; hence, the ceramic heater 1 has enhanced durability.

When leads 5 each have the two recessed portions 9, the connecting portions 3a, which are located in the recessed portions 9, preferably have substantially the same cross-sectional area. This allows the difference between the heat generated from one of the heat-generating resistors 3 and the heat generated from the other one to be reduced; hence, the difference between thermal stresses can be reduced.

In the above embodiments, the heat-generating resistors 3 preferably have a resistivity greater than the resistivity of the leads 5. When the heat-generating resistors 3 have a resistivity greater than the resistivity of the leads 5, the resistance of the heat-generating resistors 3 can be adjusted to be greater than the resistance of the leads 5 without increasing the size of the heater 1. This allows the heat-generating resistors 3 to efficiently generate heat, thereby allowing the rapid heating of the ceramic heater 1. Furthermore, the cathode-side electrodes 11 and the anode-side electrodes 13 can be prevented from being increased in temperature; hence, properties of the heater 1 can be enhanced. The heat-generating resistors 3 can be measured for resistivity as described below.

When the cross-sectional area of each heat-generating resistor 3 is constant in the plane perpendicular to the longitudinal direction, the heat-generating resistor 3 is measured for resistance (mΩ), cross-sectional area (mm²), and length (mm). The resistance thereof can be measured with a milliohm meter such as Hioki 3541 Resistance HiTester.

When the cross-sectional area of the heat-generating resistor 3 is not constant in the plane perpendicular to the longitudinal direction, the heat-generating resistor 3 may be machined with a surface grinder so as to have a shape with a cross-sectional area constant in an arbitrary direction. A useful example of the surface grinder is a surface grinder equipped with a KSK-type #250 diamond wheel available from Okamoto Kosaku Kikai. Examples of such a shape with a cross-sectional area constant in an arbitrary direction include a prismatic shape and a cylindrical shape.

The machined heat-generating resistor 3 may be measured for resistance (mΩ), cross-sectional area (mm²), and length (mm). The resistivity ρ (Ω·µm) (= resistance × cross-sectional area / length) thereof can be determined from the resistance, cross-sectional area, and length thereof. The lead 5 can be determined for resistivity by substantially the same method as that used to determine the resistivity of the heat-generating resistor 3.

The connecting portion 3a is preferably entirely located in the recessed portion 9. When the connecting portion 3a is entirely located in the recessed portion 9, the possibility of the formation of bump on the connecting portion 3a can be reduced. This results in that the formation of a crack near the connecting portion 3a is controlled; hence, the ceramic heater 1 has high durability and reliability. The fact that the connecting portion 3a is entirely located in the recessed portion 9 means that the recessed portion 9 has a depth D greater than the thickness L2 of the connecting portion 3a.

The heat-generating resistor 3 comprises the main heat-generating portion 3b and the connecting portion 3a located at the end of the main heat-generating portion 3b. The main heat-generating portion 3b preferably has a small thickness relatively to the width thereof, that is, the main heat-generating portion 3b is preferably flat in cross section perpendicular to the longitudinal direction. This allows the main heat-generating portion 3b to have a large perimeter in cross section perpendicular to the longitudinal direction and also allows the main heat-generating portion 3b to have a small thickness; hence, printing can be readily performed. Therefore, printing yield can be increased.

In particular, the main heat-generating portion 3b preferably has an elliptical shape, with the minor axis in the thickness direction, in cross section perpendicular to the longitudinal direction. When the main heat-generating portion 3b has such a shape, the main heat-generating portion 3b has a large width and a small thickness. When the main heat-generating portion 3b is elliptical in cross section, the main heat-generating portion 3b has curved surfaces; hence, thermal stresses can be prevented from being locally concentrated on the main heat-generating portion 3b.

The main heat-generating portion 3b preferably has substantially a uniform width. When the main heat-generating portion 3b is uniform in width, the main heat-generating portion 3b can be readily formed; hence, printing yield can be increased. Furthermore, locally generating heat in narrow portions thereof is controlled; hence, the ceramic heater 1 has enhanced durability. In particular, the narrowest portion of the main heat-generating portion 3b preferably has a width equal to 70% or more of that of the widest portion of the main heat-generating portion 3b. When the narrowest portion has a width equal to 70% or more of that of the widest portion, locally generating heat in narrowest portions is controlled.

The main heat-generating portion 3b preferably has substantially a uniform thickness. When the main heat-generating portion 3b is uniform in thickness, the main heat-generating portion 3b can be readily formed; hence, printing yield can be increased. Furthermore, locally generating heat in thin portion thereof is controlled; hence, the ceramic heater 1 has enhanced durability. In particular, the thinnest portion of the main heat-generating portion 3b preferably has a thickness equal to 80% or more of that of the thickest portion of the main heat-generating portion 3b. When the thinnest portion has a width equal to 80% or more of that of the thickest portion, locally generating heat in the thinnest portion is controlled.

A glow plug according to this embodiment will now be described with reference to a drawing.

As shown in Fig. 9, the glow plug 15 of this embodiment comprises a ceramic heater 1 typified by that according to any one of the above embodiments, a first metal member 17 with a cylindrical shape, an end portion of the ceramic heater 1 is located in the first metal member 17, and a second metal member 19 located in the first metal member 17, spaced from the first metal member 17, and connected to the ceramic heater 1. The heater 1 also comprises a cathode-side electrode 11 on a side surface thereof and an anode-side electrode 13 at an end thereof. The cathode-side electrode 11 is electrically connected to the first metal member 17. The anode-side electrode 13 is electrically connected to the second metal member 19.

When the second metal member 19 and the first metal member 17 are supplied with electricity, the glow plug 15 of this embodiment can function as a heat source for engine starting. Since the glow plug 15 comprises the ceramic heater 1 of the above embodiments, the glow plug 15 has enhanced durability and reliability. Even if the glow plug 15 is used in cold climates, the glow plug 15 can start an engine in a shorter time as compared with conventional ones.

A method of manufacturing a ceramic heater according to this embodiment will now be described with reference to a drawing.

The method of manufacturing a ceramic heater of this embodiment comprises preparing a green form body 21 in such a manner that a first paste 4 for a heat-generating resistor 3 and a second paste 6 for a lead 5 are provided on green ceramic sheets for a ceramic body 7 and firing the green form body 21. The first paste 4 has portions (hereinafter referred to as the connecting paste portion 4a) connected to the second paste 6. The width of the connecting paste portion 4a is less than the width of the second paste 6 and the connecting paste portion 4a is located within the width of the second paste 6.

In particular, the first paste 4 is provided on the green ceramic sheets 8a and 8c by printing as shown in Fig. 10. In this operation, the first paste 4 is provided on the sheets by printing such that the width of the connecting paste portion 4a is less than the width of the second paste 6. The width of connecting portions 3a can be readily adjusted to be less than the width of the leads 5 in such a manner that plate making and a press mold are designed such that the width of the connecting paste portion 4a is less than the width of the second paste 6. A third paste 23 for an anode-side electrode 13 and a cathode-side electrode 11 may be provided on the green ceramic sheets 8a and 8c by printing.

It is preferred that grooves be formed, in advance, in portions of the green ceramic sheets 8a and 8c that are to be provided with the first paste 4 and the first paste 4 be provided in the grooves. This is effective in that a misalignment of the first paste 4 is controlled.

The second paste 6 is provided on the green ceramic sheet 8b by printing. It is preferred that a groove or hole be formed, in advance, in a portion of the green ceramic sheet 8b that is to be provided with the second paste 6 and the second paste 6 be provided in the groove or hole. This is effective in that a misalignment of the second paste 6 is controlled.

The green form body 21 is prepared in such a manner that the green ceramic sheets 8a and 8c provided with the first paste 4 and the green ceramic sheet 8b provided with the second paste 6 are stacked such that the connecting paste portion 4a are provided within the width of the second paste 6. The green form body 21 is fired at a temperature of 1650°C to 1780°C by hot pressing. This allows the ceramic heater 1 of this embodiment to be manufactured.

The formation of a bump on the connecting portion 3a is controlled by using of the ceramic heater-manufacturing method of this embodiment. This results in that the possibility of the formation of a crack in the ceramic body 7, the heat-generating resistor 3, or the lead 5 is reduced.

The ceramic heater 1, which is rectangular parallelepiped-shaped after being fired, may be subjected to centerless grinding so as to be cylindrical. The ceramic heater 1 can be manufactured so as to have such a shape as shown in Fig. 1 in such a manner that one end portion and another end portion of the ceramic heater 1 are machined with a diamond wheel machined into a desired shape in advance.

In the above embodiment, the green ceramic sheets 8a and 8c provided with the first paste 4 and the green ceramic sheet 8b provided with the second paste 6 are stacked. These sheets may be stacked as described below.

The first paste 4 is provided on the green ceramic sheets 8a and 8c by printing. The second paste 6 is provided on the green ceramic sheets 8a and 8c by printing. The green ceramic sheets 8a and 8c provided with the first paste 4 and the second paste 6 are stacked with the green ceramic sheet 8b.

In the case where the first paste 4 and the second paste 6 are provided on the green ceramic sheets 8, which are of the same type, and the green ceramic sheets 8 are then stacked, misalignment between the element comprising the first paste 4 and the element comprising the second paste 6 can be controlled.

The width of the first paste 4 is preferably adjusted such that the width of the connecting paste portions 4a is less than that of the other portion of the first paste (hereinafter referred to as the main heat-generating paste portion 4b). This is because in order to achieve a desired amount of heat, the main heat-generating portion 3b can be designed to have a small thickness by increasing the width of the main heat-generating paste portion 4b. The reduction of the thickness of the main heat-generating portion 3b allows the adhesion between the green ceramic sheets to be enhanced. When the main heat-generating portion 3b has a small thickness, the main heat-generating portion 3b can be readily printed; hence, printing yield can be increased.

In particular, the connecting paste portions 6b preferably have a width equal to 30% to 80% of the width of the main heat-generating paste portion 6a. When the connecting paste portions 6b have a width equal to 30% or more of the width of the main heat-generating paste portion 6a, the strength at the boundaries between the main heat-generating portion 3b and the connecting portions 3a can be enhanced. Furthermore, the contact area between the connecting paste portions and the second paste is increased; hence, the bonding strength between the connecting portions 3a and the leads 5 can be enhanced. When the connecting paste portions 6b have a width equal to 80% or less of the width of the main heat-generating paste portion 6a, the adhesion between the ceramic sheets can be enhanced.

It is effective that the width of the connecting paste portions 4a is less than the width of the main heat-generating paste portion 4b. This is because the difference in thickness between the main heat-generating portion 3b and the leads 5 can be reduced. Hence, a separation of the main heat-generating portion 3b and the lead 5 from the ceramic body 7 is controlled.

In particular, the connecting paste portion 4a preferably has a thickness equal to 40% to 95% of the thickness of the main heat-generating paste portion 4b. When the connecting paste portion 4a have a thickness equal to 40% or more of the thickness of the main heat-generating paste portion 4b, the bonding strength between the second paste 6 and the connecting paste portion 4a can be enhanced. When the connecting paste portion 4a have a thickness equal to 95% or less of the thickness of the main heat-generating paste portion 4b, the connecting paste portion 4a can be readily placed in recessed portion 9. This allows the connecting paste portion 4a and the second paste 6 to be securely connected to each other.

Preferably, the thickness of the connecting paste portion 4a is less than the thickness of the second paste 6. This is because the resistance of the heat-generating resistor 3 can be increased. The increase of the resistance of the heat-generating resistor 3 allows the main heat-generating portion 3b to efficiently generate heat.

In particular, the connecting paste portion 4a preferably has a thickness equal to 5% to 50% of the thickness of the second paste 6. When the connecting paste portion 4a has a thickness equal to 5% or more of the thickness of the second paste 6, the bonding strength between the second paste 6 and the connecting paste portion 4a can be enhanced. When the connecting paste portion 4a have a thickness equal to 50% or less of the thickness of the second paste 6, the connecting paste portion 4a can be entirely placed in recessed portions 9 stably. This results in that a protrusion of the connecting paste portion 4a from the recessed portion 9 is controlled effectively; hence, the possibility of the formation of a bump on the connecting portion 3a can be reduced.

It is preferred that the second paste 6 has the recessed portion 9 and the first paste 4 is connected to the second paste 6 in the recessed portion 9. When the second paste 6 has the recessed portion 9, the misalignment of the connecting paste portion 4a can be controlled; hence, the connecting paste portion 4a can be stably provided in the recessed portion 9.

The recessed portion 9 can be formed by press molding using, for example, a mold with a predetermined shape. In particular, the following mold may be used: a mold designed such that the recessed portion 9 is formed in end portions of the second paste 6 so as to be open in the longitudinal direction and the thickness direction.

The lead 5 can be formed so as to have the recessed portion 9, which are open in the longitudinal direction and the thickness direction, in such a manner that the second paste 6 press-molded with the mold is provided on the green ceramic sheets 8 and then fired.

The present invention is not limited to the above embodiments. Various modifications may be made within the scope of the present invention.

### Examples

The ceramic heater 1 of the above embodiment was prepared as described below. A mixture was prepared by adding an oxide of Yb and MoSi₂ to a powder made of silicon nitride (Si₃N₄) as a main component. The Yb oxide was used as a sintering aid. MoSi₂ was used to adjust the thermal expansion coefficient of green ceramic sheets close to the thermal expansion coefficient of heat-generating resistors 3 and leads 5. The mixture was press-molded into the green ceramic sheets 8.

The first paste 4, the second paste 6, and the third paste 23 for an electrode lead portions were prepared. For adhesion enhancement, the first paste 4, the second paste 6, and the third paste 23 prepared from the same material made of WC and boron nitride as a main component. The first paste 4 and third paste 23 were provided on the green ceramic sheets 8 by printing.

In this operation, the first paste 4 was provided thereon so as to vary in width and thickness as shown in Table 1 below. In particular, the first paste 4 was provided thereon such that a main heat-generating portion 3b had a width of 0.6 to 1.0 mm and a thickness of 0.10 to 0.25 mm and connecting portions 3a had a width of 0.6 to 1.0 mm and a thickness of 0.07 to 0.19 mm.

The second paste 6 was provided on the green ceramic sheets 8 by printing. In this operation, the second paste 6 was provided thereon such that the leads 5 had a width of 1.0 mm and a thickness of 1.0mm. In Samples 3 to 15, recessed portions 9 were formed in end portions of the leads 5 with a press mold so as to be open in the longitudinal direction and the thickness direction, the end portions being connected to the connecting portions 3a. The recessed portions 9 had a depth D of 0.20 mm. The recessed portions 9 were quadrilateral (Fig. 2A), tapered (Fig. 5), curved (Fig. 6), or substantially arced (Fig. 7A).

The green ceramic sheets 23 provided with the second paste 6 were deposited on the green ceramic sheets 8 provided with the first paste 4 and the third paste 23. Green form body 21 was prepared as described above.

Each green form body 21 was provided in a cylindrical carbon mold and then fired at a temperature of 1650°C to 1780°C and a pressure of 30 to 50 MPa in a reducing atmosphere by hot pressing, whereby a sintered body was obtained. Electrode metal members were brazed to a cathode-side electrode 11 and anode-side electrode 13 exposed at the surface of the sintered body, whereby the ceramic heater 1 was prepared.

In this example, the heat-generating resistors 3 and the leads 5 were measured for resistivity by a procedure below. Sintered bodies were prepared from a material for forming the heat-generating resistors 3 and a material for forming the leads 5. Each sintered body was ground into a 3-mm square prism with a length of 18 mm using a surface grinder equipped with a #250 diamond wheel. Electrodes were formed on both end surfaces of the sintered body by printing and then baked in a vacuum furnace.

The sintered body was measured for resistance R (mΩ) with Hioki 3541 Resistance HiTester in such a manner that a constant current was applied between the electrodes at room temperature. $The resistivity ρ \left(Ω ⋅ μm\right) \left(= resistance \left(R\right) \times cross-sectional area / length = R / 2\right)$ thereof was calculated from the resistance thereof.

In this example, the heat-generating resistors 3 had a resistivity of 1.6 to 2.5 Ω·µm and the leads 5 had a resistivity of 2.5 Ω·µm. The reason why these sintered bodies were prepared from the material for forming the heat-generating resistors 3 in this example is to readily measure the resistivity.

Table 1 summarizes the width, thickness, and resistivity of the main heat-generating portions 3b, connecting portions 3a, and leads 5 of the samples.

**[Table 1]**

| Samples | Heat-generating resistors | | | | | Leads | | |
|---|---|---|---|---|---|---|---|---|
| | Main heat-generating portions | | Connecting portions | | Resistivity (Ω·µm) | Width (mm) | Thickness (mm) | Resistivity (Ω·µm) |
| | Width (mm) | Thickness (mm) | Width (mm) | Thickness (mm) | | | | |
| 1 | 1.0 | 0.15 | 1.0 | 0.15 | 1.6 | 1.0 | 1.0 | 2.5 |
| 2 | 1.0 | 0.10 | 1.0 | 0.10 | 2.0 | 1.0 | 1.0 | 2.5 |
| 3 | 1.0 | 0.10 | 0.8 | 0.13 | 2.0 | 1.0 | 1.0 | 2.5 |
| 4 | 0.6 | 0.25 | 0.8 | 0.19 | 1.6 | 1.0 | 1.0 | 2.5 |
| 5 | 1.0 | 0.10 | 0.8 | 0.07 | 2.0 | 1.0 | 1.0 | 2.5 |
| 6 | 1.0 | 0.10 | 0.6 | 0.07 | 2.0 | 1.0 | 1.0 | 2.5 |
| 7 | 1.0 | 0.13 | 0.8 | 0.10 | 2.5 | 1.0 | 1.0 | 2.5 |
| 8 | 1.0 | 0.10 | 0.6 | 0.07 | 2.0 | 1.0 | 1.0 | 2.5 |
| 9 | 1.0 | 0.10 | 0.6 | 0.07 | 2.0 | 1.0 | 1.0 | 2.5 |
| 10 | 1.0 | 0.10 | 0.6 | 0.07 | 2.0 | 1.0 | 1.0 | 2.5 |
| 11 | 1.0 | 0.20 | 0.6 | 0.15 | 1.6 | 1.0 | 1.0 | 2.5 |
| 12 | 1.0 | 0.15 | 0.6 | 0.10 | 1.6 | 1.0 | 1.0 | 2.5 |
| 13 | 0.8 | 0.10 | 0.8 | 0.10 | 1.6 | 1.0 | 1.0 | 2.5 |
| 14 | 0.6 | 0.11 | 0.6 | 0.11 | 1.6 | 1.0 | 1.0 | 2.5 |
| 15 | 1.0 | 0.10 | 0.6 | 0.07 | 2.0 | 1.0 | 1.0 | 2.5 |

The ceramic heater 1 was subjected to a heat cycle durability test below. The ceramic heater 1 was supplied with electricity for 30 seconds, whereby the ceramic body 7 was heated such that the surface temperature of the ceramic body 7 was increased from room temperature up to 1300°C. The resulting ceramic heater 1 was air-cooled for 60 seconds, whereby the surface temperature of the ceramic body 7 was decreased to room temperature. The ceramic heater 1 was heated and cooled for 140000 cycles. The surface temperature of the ceramic body 7 may be measured with a radiation thermometer. The resistance of the ceramic heater 1 was adjusted such that the voltage applied to the ceramic heater 1 to maintain the ceramic heater 1 at 1300°C was 190 to 210 V.

As shown in Tables 1 and 2 below, samples comprise main heat-generating portions 3b and connecting portions 3a having different widths, thicknesses, resistivities, and shapes were evaluated for printing yield. The fired samples were evaluated for cracks. The samples subjected to the heat cycle test were evaluated for cracks. The samples were observed with an optical microscope at a magnification of 450 times whether cracks were present or not.

Forty ceramic heaters 1, having a thickness of 2 mm, a width of 6 mm, and a length of 50 mm, for test use were prepared for each sample. Twenty of the heaters were fired by hot pressing and then evaluated for cracks, whereby the incidence of cracks was determined. The remaining 20 heaters subjected to the heat cycle durability test and then evaluated for cracks, whereby the incidence of cracks was determined. The evaluation results are summarized in Table 2.

**[Table 2]**

| Samples | Recessed portions | Shape of recessed portions | Arrangement of recessed portions | State of heat-generating resistors located in recessed portions | Bumps | Printing yield (%) | Crack incidence | |
|---|---|---|---|---|---|---|---|---|
| | | | | | | | Fired (%) | Evaluated for durability (%) |
| 1 | Not present | | | | Present | 80 | 70 | 80 |
| 2 | Not present | | | | Present | 100 | 60 | 65 |
| 3 | Present | Substantially arced | Opposed | Partly | Not present | 90 | 20 | 5 |
| 4 | Present | Substantially arced | Opposed | Partly | Not present | 60 | 20 | 20 |
| 5 | Present | Substantially arced | Opposed | Entirely | Not present | 100 | 0 | 0 |
| 6 | Present | Substantially arced | Opposed | Entirely | Not present | 100 | 0 | 0 |
| 7 | Present | Substantially arced | Opposed | Entirely | Not present | 85 | 0 | 5 |
| 8 | Present | Quadrilateral | Opposed | Entirely | Not present | 100 | 20 | 15 |
| 9 | Present | Trapezoidal | Opposed | Entirely | Not present | 100 | 20 | 10 |
| 10 | Present | Curved | Opposed | Entirely | Not present | 100 | 0 | 0 |
| 11 | Present | Substantially arced | Opposed | Partly | Not present | 70 | 15 | 20 |
| 12 | Present | Substantially arced | Opposed | Entirely | Not present | 80 | 0 | 0 |
| 13 | Present | Substantially arced | Opposed | Entirely | Not present | 100 | 10 | 10 |
| 14 | Present | Substantially arced | Opposed | Entirely | Not present | 100 | 10 | 10 |
| 15 | Present | Substantially arced | One-sided | Entirely | Not present | 100 | 15 | 20 |

As is clear from the results shown in Tables 1 and 2, Samples 1 and 2 have sharp wedge-shaped bumps protruding in the width direction because the connecting portions 3a of the heat-generating resistors 3 were formed so as to have the same width as that of the leads 5. Therefore, the ceramic body 7 has a high crack incidence of 60% or more.

On the other hand, the ceramic heaters 1 of Samples 3 to 15 have a crack incidence of 20% or less. This confirms that a crack incidence thereof is greatly improved because the connecting portions 3a have a width less than that of the leads 5 and therefore the thermal stresses applied thereto are reduced.

In Samples 5 to 7, 10, and 12, the recessed portions 9 are curved or substantially arced, the leads have the recessed portions located in end portions which are connected to the connecting portions and which are opposed to each other, and the connecting portions are entirely located in the recessed portions. Cracks are hardly present in Samples 5 to 7, 10, and 12, which are fired or subjected to the durability test. This shows that the ceramic heaters have significantly enhanced durability.

Samples 4 and 11, in which the main heat-generating portions 3b have a large thickness, have a relatively small printing yield of 60% to 70%. This is probably because, since the main heat-generating portions 3b have a large thickness and therefore are forced to be printed, the difference in thickness therebetween is large. In particular, Sample 4, in which the connecting portions 3a have a width greater than that of the main heat-generating portion 3b, has a low printing yield of 60%. Samples 3, 4, and 11, in which the connecting portions 3a have a large thickness, have relatively high crack incidence. This is because the connecting portions 3a are badly located in the recessed portions 9 of the leads 5.

Samples 14 and 15, in which the connecting portions 3a of the heat-generating resistors 3 have the same width as that of the main heat-generating portions 3b, have an extremely large printing yield of 100%. This is because the heat-generating resistors 3, which have a constant width, are simple in shape and therefore can be readily formed.

### Brief Description of Drawings

[Fig. 1] Fig. 1 is a sectional view of a ceramic heater according to a first embodiment of the present invention, the sectional view being perpendicular to the thickness direction of the ceramic heater.
[Fig. 2A] Fig. 2A is a sectional view of the embodiment shown in Fig. 1, the sectional view being perpendicular to the longitudinal direction of leads.
[Fig. 2B] Fig. 2B is an enlarged sectional view of a connecting portion and one of the leads shown in Fig. 2A.
[Fig. 3] Fig. 3 is a sectional view of the embodiment shown in Fig. 1, the sectional view being perpendicular to the width direction thereof.
[Fig. 4] Fig. 4 is a sectional view of a modification of the embodiment shown in Fig. 1, the sectional view being perpendicular to the width direction thereof.
[Fig. 5] Fig. 5 is a sectional view of a ceramic heater according to a second embodiment of the present invention, the sectional view being perpendicular to the longitudinal direction of the ceramic heater.
[Fig. 6] Fig. 6 is a sectional view of a ceramic heater according to a third embodiment of the present invention, the sectional view being perpendicular to the longitudinal direction of the ceramic heater.
[Fig. 7A] Fig. 7A is a sectional view of a heat-generating resistor according to a modification of the embodiment shown in Fig. 6, the sectional view being perpendicular to the longitudinal direction thereof.
[Fig. 7B] Fig. 7B is an enlarged sectional view of a connecting portion and lead shown in Fig. 7A.
[Fig. 8] Fig. 8 is a sectional view of a ceramic heater according to a fourth embodiment of the present invention, the sectional view being perpendicular to the longitudinal direction of the ceramic heater.
[Fig. 9] Fig. 9 is a schematic sectional view of an exemplary glow plug according to an embodiment of the present invention.
[Fig. 10] Fig. 10 is an exploded perspective view of a green form body used in a method for manufacturing a ceramic heater according to an embodiment of the present invention.
[Fig. 11A] Fig. 11A is a sectional view of a conventional ceramic heater, the sectional view being perpendicular to the thickness direction of the conventional ceramic heater.
[Fig. 11B] Fig. 11B is a sectional view of the conventional ceramic heater, the sectional view being perpendicular to the longitudinal direction of the conventional ceramic heater. Reference Numerals

- 1: ceramic heater
- 3: heat-generating resistor(s)
- 3a: connecting portions
- 3b: main heat-generating portion(s)
- 3c: bumps
- 4: first paste
- 4a: connecting paste portions
- 4b: main heat-generating paste portion
- 5: leads
- 6: second paste
- 7: ceramic body
- 8: green ceramic sheets
- 9: recessed portions
- 11: cathode-side electrode
- 13: anode-side electrode
- 15: glow plug
- 17: first metal member
- 19: second metal member
- 21: green form body
- 23: third paste

## Claims

1. A ceramic heater (1), comprising:
a heat-generating resistor (3),
a lead (5) configured for supplying power to the heat-generating resistor (3), and
a ceramic body (7) containing the heat-generating resistor (3) and the lead (5) therein,
wherein the heat-generating resistor (3) comprises a connecting portion (3a) being connected to the lead (5) and having a width less than the width of the lead (5), and a main heat-generating portion (3b) other than the connecting portion (3a),
**characterized in that**
the lead (5) comprises a recessed portion (9) being located at an end portion of the lead (5), being connected to the connecting portion (3a), and being open at an only one side of the longitudinal direction of the lead (5) and an only one side of the thickness direction of the lead (5), and
at least a part of the connecting portion (3a) is located inside the recessed portion (9).

2. The ceramic heater (1) according to Claim 1, wherein the connecting portion (3a) has a width less than the width of the main heat-generating portion (3b).

3. The ceramic heater (1) according to Claim 1, wherein the connecting portion (3a) has a thickness less than the thickness of the main heat-generating portion (3b).

4. The ceramic heater (1) according to Claim 1, wherein the connecting portion (3a) has a thickness less than the thickness of the lead (5).

5. The ceramic heater (1) according to Claim 1, wherein a connection surface between the connecting portion (3a) and the lead (5) comprises a curved surface.

6. The ceramic heater (1) according to Claim 5, wherein a surface shape of the recessed portion (9) is substantially an arced shape in a cross section perpendicular to the longitudinal direction.

7. The ceramic heater (1) according to Claim 1, wherein the heat-generating resistor (3) has a resistivity greater than or equal to the resistivity of the lead (5).

8. The ceramic heater (1) according to Claim 1, wherein the lead (5) comprises the recessed portions (9) which are located in the end portion of the lead (5) being connected to the connecting portion (3a) and are located at opposing parts of the end portion of the lead (5) each other, and two of the heat-generating resistors (3) comprise connecting portions (3a) each being located inside a corresponding one of the recessed portions (9).

9. The ceramic heater (1) according to Claim 1, wherein the connecting portion (3a) is entirely located inside the recessed portion (9).

10. A glow plug (15), comprising:
the ceramic heater (1) according to Claim 1,
a first metal member (17) with a cylindrical shape, an end portion of the ceramic heater (1) is located in the first metal member (17), and
a second metal member (19) located inside the first metal member (17), spaced from the first metal member (17), and connected to the ceramic heater (1).

11. A method of manufacturing a ceramic heater (1 according to claim 1), the ceramic heater (1) comprises a heat-generating resistor (3), a lead (5) configured for supplying power to the heat-generating resistor (3), and a ceramic body (7) containing the heat-generating resistor (3) and the lead (5) therein, the method being **characterized by** comprising:
preparing a green form body (21) in such a manner that a first paste (4) for the heat-generating resistor (3) and a second paste (6) for the lead (5) are provided on green ceramic sheets (8) for the ceramic body (7), at least part of the first paste (4) is connected to the second paste (6); and
firing the green form body (21),
wherein a width of a portion of the first paste (4) connected to the second paste (6) is less than the width of the second paste (6) and the portion connected to the second paste (6) is located within the width of the second paste (6).

12. The method of manufacturing a ceramic heater (1) according to Claim 11, wherein the width of a portion of the first paste (4) connected to the second paste (6) is less than the width of the other portion of the first paste (4).

13. The method of manufacturing a ceramic heater (1) according to Claim 11, wherein the thickness of a portion of the first paste (4) connected to the second paste (6) is less than the thickness of the other portion of the first paste (4).

14. The method of manufacturing a ceramic heater (1) according to Claim 11, wherein the thickness of a portion of the first paste (4) connected to the second paste (6) is less than the thickness of the second paste (6) of the first paste (4).

15. The method of manufacturing a ceramic heater (1) according to Claim 11, wherein the second paste (6) comprises a recessed portion and the first paste (4) connected to the second paste (6) inside the recessed portion.

## Patentansprüche

1. Eine keramische Heizvorrichtung (1), aufweisend:
einen wärmeerzeugenden Widerstand (3),
eine Leitung (5), die konfiguriert ist, um dem wärmeerzeugenden Widerstand (3) Strom zuzuführen, und
einen Keramikkörper (7), der darin den wärmeerzeugenden Widerstand (3) und die Leitung (5) enthält,
wobei der wärmeerzeugende Widerstand (3) einen Verbindungsabschnitt (3a), der mit der Leitung (5) verbunden ist und eine Breite hat, die kleiner als die Breite der Leitung (5) ist, und einen Haupt-Wärmeerzeugungsabschnitt (3b), der anders ist als der Verbindungsabschnitt (3a), aufweist,
**dadurch gekennzeichnet, dass**
die Leitung (5) einen Aussparungsabschnitt (9) aufweist, der an einem Endabschnitt der Leitung (5) angeordnet ist, mit dem Verbindungsabschnitt (3a) verbunden ist und auf nur einer Seite der Längsrichtung der Leitung (5) und nur einer Seite der Dickenrichtung der Leitung (5) offen ist, und
mindestens ein Teil des Verbindungsabschnitts (3a) innerhalb des Aussparungsabschnitts (9) angeordnet ist.

2. Die keramische Heizvorrichtung (1) gemäß Anspruch 1, wobei der Verbindungsabschnitt (3a) eine Breite hat, die kleiner als die Breite des Haupt-Wärmeerzeugungsabschnitts (3b) ist.

3. Die keramische Heizvorrichtung (1) gemäß Anspruch 1, wobei der Verbindungsabschnitt (3a) eine Dicke hat, die kleiner als die Dicke des Haupt-Wärmeerzeugungsabschnitts (3b) ist.

4. Die keramische Heizvorrichtung (1) gemäß Anspruch 1, wobei der Verbindungsabschnitt (3a) eine Dicke hat, die kleiner als die Dicke der Leitung (5) ist.

5. Die keramische Heizvorrichtung (1) gemäß Anspruch 1, wobei eine Verbindungfläche zwischen dem Verbindungsabschnitt (3a) und der Leitung (5) eine Krümmungsfläche aufweist.

6. Die keramische Heizvorrichtung (1) gemäß Anspruch 5, wobei eine Oberflächenform des Aussparungsabschnitts (9) in einem Querschnitt senkrecht zu der Längsrichtung im Wesentlichen eine gewölbte Form ist.

7. Die keramische Heizvorrichtung (1) gemäß Anspruch 1, wobei der wärmeerzeugende Widerstand (3) eine Resistivität hat, die größer oder gleich der Resistivität der Leitung (5) ist.

8. Die keramische Heizvorrichtung (1) gemäß Anspruch 1, wobei die Leitung (5) die Aussparungsabschnitte (9) aufweist, die im Endabschnitt der Leitung (5), der mit dem Verbindungsabschnitt (3a) verbunden ist, angeordnet sind und an einander entgegengesetzten Teilen des Endabschnitts der Leitung (5) angeordnet sind, und wobei zwei der wärmeerzeugenden Widerstände (3) Verbindungsabschnitte (3a) aufweisen, die jeweils innerhalb eines der Aussparungsabschnitte (9) angeordnet sind.

9. Die keramische Heizvorrichtung (1) gemäß Anspruch 1, wobei der Verbindungsabschnitt (3a) vollständig innerhalb des Aussparungsabschnitts (9) angeordnet ist.

10. Eine Glühkerze (15), aufweisend:
die keramische Heizvorrichtung (1) gemäß Anspruch 1,
ein erstes Metallelement (17) mit einer zylindrischen Form, wobei ein Endabschnitt der keramischen Heizvorrichtung (1) in dem ersten Metallelement (17) angeordnet ist, und
ein zweites Metallelement (19), das innerhalb des ersten Metallelements (17) angeordnet ist, im Abstand von dem ersten Metallelement (17) angeordnet ist und mit der keramischen Heizvorrichtung (1) verbunden ist.

11. Ein Verfahren zum Herstellen einer keramischen Heizvorrichtung (1) gemäß Anspruch 1, wobei die keramische Heizvorrichtung (1) einen wärmeerzeugenden Widerstand (3), eine Leitung (5), die zum Zuführen von Strom an den wärmeerzeugenden Widerstand (3) konfiguriert ist, und einen Keramikkörper (7) aufweist, der darin den wärmeerzeugenden Widerstand (3) und die Leitung (5) aufweist, wobei das Verfahren **dadurch gekennzeichnet ist, dass** es aufweist:
Herstellen eines Grünkörpers (21) derart, dass eine erste Paste (4) für den wärmeerzeugenden Widerstand (3) und eine zweite Paste (6) für die Leitung (5) auf Keramik-Grünkörpern (8) für den Keramikkörper (7) vorgesehen sind, wobei zumindest ein Teil der ersten Paste (4) mit der zweiten Paste (6) verbunden ist, und
Brennen des Grünkörpers (21),
wobei eine Breite eines Abschnitts der erste Paste (4), der mit der zweiten Paste (6) verbunden ist, kleiner als die Breite der zweiten Paste (6) ist, und der Abschnitt, der mit der zweiten Paste (6) verbunden ist, innerhalb der Breite der zweiten Paste (6) angeordnet ist.

12. Das Verfahren zum Herstellen einer keramischen Heizvorrichtung (1) gemäß Anspruch 11, wobei die Breite eines Abschnitts der ersten Paste (4), der mit der zweiten Paste (6) verbunden ist, kleiner als die Breite des anderen Abschnitts der ersten Paste (4) ist.

13. Das Verfahren zum Herstellen einer keramischen Heizvorrichtung (1) gemäß Anspruch 11, wobei die Dicke eines Abschnitts der ersten Paste (4), der mit der zweiten Paste (6) verbunden ist, kleiner als die Dicke des anderen Abschnitts der ersten Paste (4) ist.

14. Das Verfahren zum Herstellen einer keramischen Heizvorrichtung (1) gemäß Anspruch 11, wobei die Dicke eines Abschnitts der ersten Paste (4), der mit der zweiten Paste (6) verbunden ist, kleiner als die Dicke der zweiten Paste (6) der ersten Paste (4) ist.

15. Das Verfahren zum Herstellen einer keramischen Heizvorrichtung (1) gemäß Anspruch 11, wobei die zweite Paste (6) einen Aussparungsabschnitt aufweist und die erste Paste (4) innerhalb des Aussparungsabschnitts mit der zweiten Paste (6) verbunden ist.

## Revendications

1. Un dispositif de chauffage en céramique (1), comportant :
une résistance génératrice de chaleur (3),
une conduite (5) configurée pour alimenter la résistance génératrice de chaleur (3) en énergie, et
un corps en céramique (7) comprenant la résistance génératrice de chaleur (3) et la conduite (5) là-dedans,
dans lequel la résistance génératrice de chaleur (3) comporte une partie de connexion (3a) étant reliée à la conduite (5) et ayant une largeur inférieure à la largeur de la conduite (5), et une partie génératrice de chaleur principale (3b) à part la partie de connexion (3a),
**caractérisé en ce que**
la conduite (5) comprend une partie en retrait (9) située à une partie terminale de la conduite (5), reliée à la partie de connexion (3a) et ouverte d'un seul côté de la direction longitudinale de la conduite (5) et d'un seul côté de la direction d'épaisseur de la conduite (5), et
au moins une partie de la partie de connexion (3a) est située à l'intérieur de la partie en retrait (9).

2. Le dispositif de chauffage en céramique (1) selon la revendication 1, dans lequel la partie de connexion (3a) a une largeur inférieure à la largeur de la partie génératrice de chaleur principale (3b).

3. Le dispositif de chauffage en céramique (1) selon la revendication 1, dans lequel la partie de connexion (3a) a une épaisseur inférieure à l'épaisseur de la partie génératrice de chaleur principale (3b).

4. Le dispositif de chauffage en céramique (1) selon la revendication 1, dans lequel la partie de connexion (3a) a une épaisseur inférieure à l'épaisseur de la conduite (5).

5. Le dispositif de chauffage en céramique (1) selon la revendication 1, dans lequel une surface de connexion entre la partie de connexion (3a) et la conduite (5) comprend une surface courbée.

6. Le dispositif de chauffage en céramique (1) selon la revendication 5, dans lequel une forme de surface de la partie en retrait (9) est essentiellement une forme en arc en section transversale perpendiculaire à la direction longitudinale.

7. Le dispositif de chauffage en céramique (1) selon la revendication 1, dans lequel la résistance génératrice de chaleur (3) a une résistivité supérieure ou égale à la résistivité de la conduite (5).

8. Le dispositif de chauffage en céramique (1) selon la revendication 1, dans lequel la conduite (5) comprend les parties en retrait (9) qui sont situées dans la partie terminale de la conduite (5) reliée à la partie de connexion (3a) et sont situées à des parties opposées les unes des autres de la partie terminale de la conduite (5), et deux parmi les résistances génératrices de chaleur (3) comprennent des parties de connexion (3a) étant chacune située à l'intérieure d'une correspondante des parties en retrait (9).

9. Le dispositif de chauffage en céramique (1) selon la revendication 1, dans lequel la partie de connexion (3a) est complètement située à l'intérieur de la partie en retrait (9).

10. Une bougie de préchauffage (15), comportant :
le dispositif de chauffage en céramique (1) selon la revendication 1,
un premier élément métallique (17) ayant une forme cylindrique, une partie terminale du dispositif de chauffage en céramique (1) étant située dans le premier élément métallique (17), et
un deuxième élément métallique (19) situé à l'intérieur du premier élément métallique (17), espacé du premier élément métallique (17) et relié au dispositif de chauffage en céramique (1).

11. Un procédé de fabrication d'un dispositif de chauffage en céramique (1) selon la revendication 1, dans lequel le dispositif de chauffage en céramique (1) comprend une résistance génératrice de chaleur (3), une conduite (5) configurée pour alimenter la résistance génératrice de chaleur (3) en énergie, et un corps en céramique (7) comprenant la résistance génératrice de chaleur (3) et la conduite (5) là-dedans, le procédé étant **caractérisé en ce qu'**il comprend les étapes consistant à :
préparer un corps vert (21) de telle façon qu'une première pâte (4) pour la résistance génératrice de chaleur (3) et une deuxième pâte (6) pour la conduite (5) sont prévues sur des feuilles céramique vertes (8) pour le corps en céramique (7), au moins une partie de la première pâte (4) étant reliée à la deuxième pâte (6), et
cuire le corps vert (21),
dans lequel une largeur d'une partie de la première pâte (4) reliée à la deuxième pâte (6) est inférieure à la largeur de la deuxième pâte (6) et la partie reliée à la deuxième pâte (6) est située dans la largeur de la deuxième pâte (6).

12. Le procédé de fabrication d'un dispositif de chauffage en céramique (1) selon la revendication 11, dans lequel la largeur d'une partie de la première pâte (4) reliée à la deuxième pâte (6) est inférieure à la largeur de l'autre partie de la première pâte (4).

13. Le procédé de fabrication d'un dispositif de chauffage en céramique (1) selon la revendication 11, dans lequel l'épaisseur d'une partie de la première pâte (4) reliée à la deuxième pâte (6) est inférieure à l'épaisseur de l'autre partie de la première pâte (4).

14. Le procédé de fabrication d'un dispositif de chauffage en céramique (1) selon la revendication 11, dans lequel l'épaisseur d'une partie de la première pâte (4) reliée à la deuxième pâte (6) est inférieure à l'épaisseur de la deuxième pâte (6) de la première pâte (4).

15. Le procédé de fabrication d'un dispositif de chauffage en céramique (1) selon la revendication 11, dans lequel la deuxième pâte (6) comprend une partie en retrait et la première pâte (4) reliée à la deuxième pâte (6) à l'intérieur de la partie en retrait.
